

# United States Patent Office

2,711,009

Patented June 21, 1955

1

2,711,009

## CORROSION RESISTANT SINTERED STOCK CONTAINING MIXED CARBIDES

John C. Redmond, Greensburg, and John W. Graham, Ligonier, Pa., assignors to Kennametal Inc., Latrobe, Pa., a corporation of Pennsylvania

No Drawing. Application October 8, 1952,  
Serial No. 313,810

3 Claims. (Cl. 29—182.7)

Our invention relates to an improved corrosion-resistant hard composition of matter and has to do, more particularly, with improvements in the corrosion-resistant hard composition of matter described and claimed in the pending application for United States Letters Patent of Philip M. McKenna, Alex G. McKenna and John C. Redmond, Serial No. 268,004, filed January 24, 1952, as a continuation-in-part of an earlier application, Serial No. 74,742, filed February 5, 1949, now abandoned.

The principal object of our invention is to provide a sintered hard composition of matter which, with the density, hardness and resistance to oxidation of the composition of said application, will have a greater transverse rupture strength at room temperature.

A primary method of evaluation of compositions, such as those disclosed in said application, has been evolved and is called the "stress-rupture test." It consists of maintaining a static tensile load on a suitable specimen at some specified elevated temperature until the specimen fails by breaking in tension in some interval of time between one and 1000 hours. By testing a series of specimens at various loads and at one temperature a graph can be drawn with time the abscissa and stress as the ordinate. When scaled properly a straight line results. The tests are generally made at several temperatures to develop a range of stress-temperature conditions. Various alloys or compositions are compared by comparing the slopes of the lines on the several graphs. A further object of our invention is to provide a sintered hard composition of matter which gives better results under the stress-rupture test.

A further object of our invention is to provide a sintered hard composition of matter having increased tensile strength and an increased modulus of elasticity.

Further objects, and objects relating to details and economies of operation, will appear more definitely from the detailed description to follow.

In general, our invention consists in substituting, for the nickel, cobalt or iron binder metal used in the compositions of said application, a binder metal consisting of an alloy of molybdenum with a metal of the iron group (nickel, cobalt or iron). The binder metal alloy should constitute from 20% to 50% of the composition, and the molybdenum should constitute from 5% to 25% of the said alloy.

The following are specific examples of compositions made in accordance with our invention.

### Example I

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 62.0     |
| Cb(TaTi)C | 8.0      |
| Ni        | 25.0     |
| Mo        | 5.0      |

2

The titanium carbide used, in this and the following examples, was substantially devoid of free titanium, free carbon, oxides and nitrides, and prepared by the method described and claimed in United States Letters Patent of Philip M. McKenna, No. 2,515,463, patented July 18, 1950. The Cb(TaTi)C used in this end and the following examples contained about 45% columbium carbide (CbC), about 42.5% tantalum carbide (TaC) and about 12.5% titanium carbide (TiC) and was made in accordance with United States Letters Patent of Philip M. McKenna, No. 2,124,509, patented July 19, 1938. The proportion of the ingredients of Cb(TaTi)C, given above, are not critical and may vary somewhat depending on the columbium ore used to make it.

The hard composition of matter made from the mix above specified, by the procedure hereinafter described, had a density of 6.06 grams per cubic centimeter, a hardness of 88.7 on the Rockwell A scale, and a transverse rupture strength at room temperature of 191,000 p. s. i. (pounds per square inch). Tests of a number of specimens of this composition showed an average tensile strength of 119,300 p. s. i. (pounds per square inch) and an average Young's modulus of elasticity between zero and maximum stress of  $57.6 \times 10^6$  p. s. i. These values were considerably higher than those for a composition that was identical except that it contained no molybdenum and 30% nickel. Specimens of the composition of Example I gave better results under the stress-rupture tests referred to above. This composition proved to be extremely resistant to corrosion or oxidation at high temperatures.

### Example II

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 57.0     |
| Cb(TaTi)C | 8.0      |
| Ni        | 30.0     |
| Mo        | 5.0      |

The hard composition of matter made from the mix above specified, by the procedure hereinafter described, had a density of 6.2 grams per cubic centimeter, a hardness of 86.7 on the Rockwell A scale, and a transverse rupture strength at room temperature of 177,000 p. s. i. Specimens of the composition of Example II gave better results under the stress-rupture test referred to above than compositions not containing molybdenum and otherwise like this composition. The composition above described proved to be extremely resistant to corrosion or oxidation at high temperatures.

### Example III

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 62.0     |
| Cb(TaTi)C | 8.0      |
| Ni        | 28.5     |
| Mo        | 1.5      |

The hard composition of matter made from the mix above specified, by the procedure hereinafter described, had a density of 6.05 grams per cubic centimeter, a hardness of 86.9 on the Rockwell A scale, and a transverse rupture strength at room temperature of 155,000 p. s. i.

## 3

This composition proved to be extremely resistant to corrosion or oxidation at high temperatures.

## Example IV

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 62.0     |
| Cb(TaTi)C | 8.0      |
| Ni        | 22.5     |
| Mo        | 7.5      |

The hard composition of matter made from the mix above specified, by the procedure hereinafter described, had a density of 6.02 grams per cubic centimeter, a hardness of 90.0 on the Rockwell A scale, and a transverse rupture strength at room temperature of 173,750 p. s. i. (pounds per square inch). Specimens of this composition proved to be extremely resistant to corrosion or oxidation at high temperatures.

## Example V

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 72.0     |
| Cb(TaTi)C | 8.0      |
| Ni        | 16.7     |
| Mo        | 3.3      |

The hard composition of matter made from the mix above specified, by the procedure hereinafter described, had a density of 5.60 grams per cubic centimeter, a hardness of 89.5 on the Rockwell A scale, and a transverse rupture strength at room temperature of 156,000 p. s. i. (pounds per square inch). Specimens of this composition gave improved results under the above-mentioned stress-rupture tests and the composition proved to be extremely resistant to corrosion or oxidation at high temperatures.

## Example VI

This composition consisted of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 72.0     |
| Cb(TaTi)C | 8.0      |
| Ni        | 15.0     |
| Mo        | 5.0      |

The hard composition of matter made from the mix above specified, by the procedure hereinafter described, had a density of 5.75 grams per cubic centimeter, a hardness of 91.8 on the Rockwell A scale, and a transverse rupture strength at room temperature of 152,800 p. s. i. (pounds per square inch). Specimens of this composition gave improved results under the stress-rupture tests referred to above and the composition proved to be extremely resistant to corrosion or oxidation at high temperatures.

## Example VII

This composition consists of titanium carbide (TiC), a complex carbide solid solution containing columbium, tantalum, titanium and carbon and referred to herein as

## 4

Cb(TaTi)C, nickel and molybdenum, in the following proportions, by weight:

|           | Per cent |
|-----------|----------|
| TiC       | 55.0     |
| Cb(TaTi)C | 15.0     |
| Ni        | 27.0     |
| Mo        | 3.0      |

The hard composition of matter made from the mix above specified, by the procedure hereinafter described, had a density of 6.30 grams per cubic centimeter, a hardness of 87.0 on the Rockwell A scale, and a transverse rupture strength at room temperature of 172,000 p. s. i. (pounds per square inch). Specimens of this composition proved to be extremely resistant to corrosion or oxidation at high temperatures.

## Example VIII

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 55.0     |
| Cb(TaTi)C | 15.0     |
| Ni        | 28.5     |
| Mo        | 1.5      |

The hard composition of matter made from the mix above specified, by the procedure hereinafter described, had a density of 6.22 grams per cubic centimeter, a hardness of 86.3 on the Rockwell A scale, and a transverse rupture strength at room temperature of 150,000 p. s. i. (pounds per square inch). This composition proved to be extremely resistant to corrosion or oxidation at high temperatures.

## Example IX

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 56.0     |
| Cb(TaTi)C | 4.0      |
| Ni        | 30.0     |
| Mo        | 10.0     |

The hard composition of matter made from the mix above specified, by the procedure hereinafter described, had a density of 6.24 grams per cubic centimeter, a hardness of 87.5 on the Rockwell A scale, and a transverse rupture strength at room temperature of 216,000 p. s. i. (pounds per square inch). Specimens of this composition proved to be resistant to corrosion or oxidation at high temperatures although not so resistant as the compositions previously described.

## Example X

This composition consists of titanium carbide (TiC), a complex carbide solid solution containing columbium, tantalum, titanium and carbon and referred to herein as Cb(TaTi)C, nickel and molybdenum, in the following proportions, by weight:

|           | Per cent |
|-----------|----------|
| TiC       | 66.0     |
| Cb(TaTi)C | 4.0      |
| Ni        | 28.5     |
| Mo        | 1.5      |

The hard composition of matter made from the mix above specified, by the procedure hereinafter described, had a density of 5.92 grams per cubic centimeter, a hard-

ness of 85.9 on the Rockwell A scale, and a transverse rupture strength of 206,000 p. s. i. (pounds per square inch). The resistance to corrosion or oxidation at high temperatures of this composition is good, although not quite as good as that of the compositions of Examples I to VIII, inclusive.

*Example XI*

This composition consists of titanium carbide (TiC), a complex carbide solid solution containing columbium, tantalum, titanium and carbon and referred to herein as  $\text{Cb}(\text{TaTi})\text{C}$ , nickel and molybdenum, in the following proportions, by weight:

|                                  | Per cent |
|----------------------------------|----------|
| TiC                              | 66.0     |
| $\text{Cb}(\text{TaTi})\text{C}$ | 4.0      |
| Ni                               | 27.0     |
| Mo                               | 3.0      |

The hard composition of matter made from the mix above specified, by the procedure hereinafter described, had a density of 6.82 grams per cubic centimeter, a hardness of 87.2 on the Rockwell A scale, and a transverse rupture strength at room temperature of 169,500 p. s. i. (pounds per square inch). The resistance of specimens of this composition to corrosion or oxidation at high temperatures was found to be good as compared with the compositions of Examples I to VII, inclusive, which were classified as very good.

*Example XII*

This composition consists of titanium carbide (TiC), a complex carbide solid solution containing columbium, tantalum, titanium and carbon and referred to herein as  $\text{Cb}(\text{TaTi})\text{C}$ , nickel and molybdenum, in the following proportions, by weight:

|                                  | Per cent |
|----------------------------------|----------|
| TiC                              | 66.0     |
| $\text{Cb}(\text{TaTi})\text{C}$ | 4.0      |
| Ni                               | 25.0     |
| Mo                               | 5.0      |

The hard composition of matter made from the mix above specified, by the procedure hereinafter described, had a density of 5.91 grams per cubic centimeter, a hardness of 89.2 on the Rockwell A scale, and a transverse rupture strength at room temperature of 174,000 p. s. i. (pounds per square inch). Specimens of this composition gave improved results under the stress-rupture tests referred to above. This composition proved to have a resistance to corrosion or oxidation at high temperatures that was classified as good as compared with the resistance to corrosion and oxidation of Examples I to VIII, inclusive, which was characterized as very good.

*Example XIII*

This composition consists of titanium carbide (TiC), a complex carbide solid solution containing columbium, tantalum, titanium and carbon and referred to herein as  $\text{Cb}(\text{TaTi})\text{C}$ , nickel and molybdenum, in the following proportions, by weight:

|                                  | Per cent |
|----------------------------------|----------|
| TiC                              | 42.0     |
| $\text{Cb}(\text{TaTi})\text{C}$ | 8.0      |
| Ni                               | 40.0     |
| Mo                               | 10.0     |

The hard composition of matter made from the mix above specified, by the procedure hereinafter described, had a density of 6.80 grams per cubic centimeter, a hardness of 83.6 on the Rockwell A scale, and a transverse rupture strength at room temperature of 202,000 p. s. i. (pounds per square inch). The resistance to corrosion or oxidation at high temperatures of specimens of this

75 The sintering temperatures used in producing the com-

composition, however, were characterized as good to poor.

*Example XIV*

This composition consists of titanium carbide (TiC), a complex carbide solid solution containing columbium, tantalum, titanium and carbon and referred to herein as  $\text{Cb}(\text{TaTi})\text{C}$ , nickel and molybdenum, in the following proportions, by weight:

|                                  | Per cent |
|----------------------------------|----------|
| TiC                              | 52.0     |
| $\text{Cb}(\text{TaTi})\text{C}$ | 8.0      |
| Ni                               | 25.0     |
| Mo                               | 15.0     |

The hard composition of matter made from the mix above specified, by the procedure hereinafter described, had a density of 6.56 per cubic centimeter, a hardness of 89.6 on the Rockwell A scale, and a transverse rupture strength at room temperature of 175,500 p. s. i. (pounds per square inch). However, the resistance to corrosion or oxidation at high temperatures of specimens of this composition was found to be poor.

The compositions of matter above described may be made by the method usually used for making cemented carbide tool compositions except that certain refinements are desirable for producing the best results. The carbide constituents of the composition, in the form of crystals passing through a sieve having 100 meshes to the inch, and the powdered or auxiliary metal (nickel and molybdenum), having an average particle size of about 25 microns, are charged into a steel ball mill. The balls used in the mill may be either cemented carbide or steel, since the presence of iron in these compositions is not deleterious. The ball mill is then filled with a light petroleum solvent to exclude the air therefrom and is thereupon sealed, and the charge is ball-milled for from three to six days, at the end of which time the liquid in the mill and charge is removed by decantation and evaporation and a temporary binder, such as 0.25 to 1.00% of paraffin, is incorporated with the material. The average particle size of the material, at the end of the ball-milling operation, is from 1 to 5 microns. The mixture is next pressed to the desired shape, or as near to it as feasible.

Although this may be done by any conventional pressing method, we have found that much more desirable results are obtained by the use of the explosive pressing process, described and claimed in the spending application for United States Letters Patent of Philip M. McKenna, John C. Redmond and Emlyn N. Smith, Serial No. 766,570, filed August 6, 1947, entitled Explosive Pressing of Powdered Compositions, upon which U. S. Letters Patent No. 2,648,125 were granted on August 11, 1953. According to this process pressure is applied to the material hydrostatically and rapidly from all directions and very high pressures may be so applied. After pressing the mixture to the desired form, the pieces may thereupon be sintered, or they may be further shaped by machining operations and, then, sintered. However, if any very complex shape is required, the material in this form has insufficient strength to withstand the necessary machining operations and, in that case, it is given a preliminary heat treatment at temperatures of from 1900° to 2100° F. to give it sufficient strength to withstand the pressure of machining or working with diamond tools, but such heat treatment is not sufficient to effect the sintering. After final shaping, in which proper allowance must be made for shrinkage during sintering, amounting to from 16 to 20%, the final sintering is carried out at temperatures of 2400° to 3000° F. in an electric induction furnace, in which a vacuum of 100 microns or less is maintained throughout the sintering operation. After the cooling of the furnace, the pieces may be removed therefrom and brought to final shape, as may be required, by grinding with a diamond wheel.

70 The sintering temperatures used in producing the com-

positions of Examples I to XIV, inclusive, are as shown by the following tabulation:

| Example  | Sintering Temperature, ° F. | Example   | Sintering Temperature, ° F. |
|----------|-----------------------------|-----------|-----------------------------|
| I.....   | 2,450                       | VIII..... | 2,600                       |
| II.....  | 2,500                       | IX.....   | 2,450                       |
| III..... | 2,500                       | X.....    | 2,700                       |
| IV.....  | 2,700                       | XI.....   | 2,600                       |
| V.....   | 2,600                       | XII.....  | 2,520                       |
| VI.....  | 2,600                       | XIII..... | 2,500                       |
| VII..... | 2,450                       | XIV.....  | 2,800                       |

It is our belief that at the sintering temperatures employed the nickel and molybdenum alloy so that the metal binding the carbide particles of the composition together is an alloy of nickel and molybdenum. The remaining metals of the iron group, that is, cobalt and iron, are equivalents of nickel for use in the making of these hard compositions of matter and cobalt or iron may be substituted for the nickel in the above compositions.

To determine the resistance of the compositions to oxidation and corrosion at high temperatures oxidation tests at 1800° F. were made on the specimens in eleven eighteen-hour increments for a total time of 198 hours. Those compositions which withstood the complete test of 198 hours with no more than .003 inch of adherent oxide growth per face were classified as excellent. Such compositions usually oxidized in a decreasing parabolic rate indicative of self protection and long life under severe oxidizing conditions. Those compositions which have the decreasing parabolic rate type of oxidation resistance or a slow linear rate and in which an inherent oxide coating forms that is greater than .003 inch and less than .008 inch in 198 hours are classified as good with respect to resistance to oxidation or corrosion at high temperatures. Those compositions which oxidize to a greater extent than .010 inch per face under the conditions specified above, or which develop a loose, flaky or powdery coating but which do not lose shape in 198 hours are classified as poor with respect to resistance to oxidation or corrosion at high temperatures.

From the foregoing examples it will be seen that compositions containing from 42 to 72% TiC, from 4 to 15% Cb(TaTi)C and from 20 to 50% of a binder metal alloy of nickel and molybdenum in which the molybdenum constitutes from 5 to 25% of the alloy have very desirable characteristics. The most desirable characteristics appear to be those of compositions including from 55 to 72% TiC, from 8 to 15% Cb(TaTi)C and from 20 to 35% of a binder metal alloy of nickel and molybdenum in which the molybdenum constitutes from 5 to 25% of the alloy.

We are aware that the compositions of matter herein described are susceptible of considerable variation from the specific proportions shown without departing from the

spirit of our invention and, therefore, we claim our invention broadly as indicated by the appended claims.

Having thus described our invention, what we claim as new and useful, and desire to secure by United States Letters Patent, is:

- 5 1. A corrosion-resistant sintered hard composition of matter consisting of from 42% to 72% titanium carbide (TiC), substantially devoid of free titanium, free carbon, oxides and nitrides, from 4% to 15% of a complex carbide solid solution containing columbium, tantalum, titanium and carbon, and from 20% to 50% of a binder metal alloy of nickel and molybdenum, in which the molybdenum constitutes from 5% to 25% of the alloy, said composition being characterized by a density of from 5.6 to 6.8 grams per cubic centimeter, a hardness on the Rockwell A scale exceeding 83.5, a transverse rupture strength, at room temperature, greater than 150,000 p. s. i. (pounds per square inch), and high resistance to oxidation at temperatures of 1800° F. and above.
- 10 2. A corrosion-resistant sintered hard composition of matter consisting of from 55% to 72% titanium carbide (TiC), substantially devoid of free titanium, free carbon, oxides and nitrides, from 8% to 15% of a complex carbide solid solution containing columbium, tantalum, titanium and carbon, and from 20% to 35% of a binder metal alloy of nickel and molybdenum, in which the molybdenum constitutes from 5% to 25% of the alloy, said composition being characterized by a density of from 5.6 to 6.3 grams per cubic centimeter, a hardness on the Rockwell A scale exceeding 86, a transverse rupture strength, at room temperature, greater than 150,000 pounds per square inch, and high resistance to oxidation at temperatures of 1800° F. and above.
- 15 3. A corrosion-resistant hard composition of matter consisting of about 62% titanium carbide (TiC), substantially devoid of free titanium, free carbon, oxides and nitrides, about 8% of a complex carbide solid solution containing columbium, tantalum, titanium and carbon, and about 30% of a binder metal alloy of nickel and molybdenum, in which the molybdenum constitutes about 15% of the alloy, characterized by a density of about 6 grams per cubic centimeter, a hardness on the Rockwell A scale of about 88.7, a transverse rupture strength at room temperature, of about 191,000 p. s. i., and high resistance to oxidation at temperatures of 1800° F. and above.
- 20
- 25
- 30
- 35
- 40
- 45

References Cited in the file of this patent

UNITED STATES PATENTS

|           |             |               |
|-----------|-------------|---------------|
| 2,023,413 | Fetkenheuer | Dec. 10, 1935 |
| 2,106,162 | Balke       | Jan. 25, 1938 |
| 2,124,509 | McKenna     | July 19, 1938 |
| 2,147,329 | Willey      | Feb. 14, 1939 |